

# UNITED STATES PATENT OFFICE.

JAMES E. ATWOOD, OF WORCESTER, MASSACHUSETTS.

## IMPROVEMENT IN MALLEABLE-IRON CASTINGS.

Specification forming part of Letters Patent No. **221,996**, dated November 25, 1879; application filed November 12, 1878.

*To all whom it may concern:*

Be it known that I, JAMES E. ATWOOD, of the city of Worcester, in the county of Worcester and State of Massachusetts, have invented a new and Improved Mixture of Irons for White-Hearted Malleable-Iron Castings, of which the following is a specification.

This invention has for its object to reduce the time, labor, and expense of manufacturing malleable cast-iron, and to produce an improved malleable cast-iron, which may be distinguished from all other malleable cast-iron by its great density, which is nearly equal to that of hammered cast-steel, and by its tensile strength, which is about double that of the ordinary malleable cast-iron; and, further, by its ability to resist rust and receive a high polish, the facility with which it may be case-hardened, and the absence of all tendency to become laminated or threaded or clawed up when being forged, like the ordinary malleable iron, during the operation of forging.

Heretofore malleable cast-iron has been produced by decarbonizing, to a proper extent, ordinary cast-iron, involving a process requiring much time and labor.

By my improved process the amount of time and labor necessary to produce the iron is greatly diminished and a superior iron is produced.

To this end the invention consists in an improved white-hearted malleable iron produced by mixing ordinary pig-iron and wrought-iron, either alone or in combination, with sprue, scoria, or dross, and fusing the same together and subjecting the mass to the action of the atmosphere, as more fully hereinafter specified.

The proportions of these materials may be varied considerably, according to the particular purpose for which the resultant product is to be used; but for general purposes I have found that equal parts of carburet or pig iron and decarbonized or wrought iron answer well in practice with one part of sprue to every two parts of decarbonized iron. The materials are properly mixed and placed in an ordinary reverberatory or other suitable furnace, and maintained in a state of fusion for a proper time—about one hour and a quarter for one ton—and subjecting it in the meantime to the influence of the atmosphere, by which the carbon is burned out to a proper extent, the product being a fine-grained and very dense iron, which may be readily cast, and is particularly adapted to the manufacture of small articles, such as harness-mountings, buckles, carriage-wheel fenders, pistol-frames, and the like, although it will answer equally well for larger articles.

I am aware that wrought-iron and pig-iron have been combined by fusion for the manufacture of steel, and this I do not claim; but

What I do claim is—

An article of manufacture consisting of a white-hearted malleable iron possessing the density of hammered steel and a tensile strength of about double that of the ordinary malleable iron, as set forth.

JAMES E. ATWOOD.

Witnesses:

A. T. MATTHEWS,  
WILLIAM BUCKLEY.